

# UNITED STATES PATENT OFFICE.

FRANCIS I. DU PONT AND ERNEST DU PONT, OF WILMINGTON, DELAWARE.

PERFORATED PELLET OF EXPLOSIVE POWDER AND PROCESS OF MAKING SAME.

1,352,121.

Specification of Letters Patent.

Patented Sept. 7, 1920.

No Drawing.

Application filed June 12, 1918. Serial No. 239,530.

To all whom it may concern:  
Be it known that we, FRANCIS I. DU PONT and ERNEST DU PONT, citizens of the United States, residing at Wilmington, county of 5 New Castle, and State of Delaware, have invented a new and useful Improvement in Perforated Pellets of Explosive Powder and Processes of Making Same, of which the following is a full, clear, and exact description.

In the manufacture of perforated pellets of explosive powder for communication trains in shrapnel shells and for similar purposes, it is necessary, for reasons well known to those skilled in the art, that there be a continuous opening through these communication trains. This is generally accomplished by compressing black powder in molds which form small perforated cylinders and building up a train of these cylinders to the desired length.

Our method of making these communication trains consists in thoroughly mixing black powder, which should be in the form of dust, with a collodion comprising nitrocellulose dissolved in alcohol and ether, or nitroglycerin and nitrocellulose dissolved in alcohol, ether and acetone. The mixing operation may be conducted in a mixing machine of the type ordinarily used in the manufacture of smokeless powder. After mixing, the powder is formed into tubes of the desired diameter having perforations of the desired size. This may be conveniently done by pressing the powder out in a macaroni press. The tubes may be cut, before drying, to form pellets similar to those now in use, or they may be cut to correspond to the length of the train or to any shorter length desired. When dried, the effect of the collodion is to cement the powder together so that a mass is produced sufficiently hard for the purpose.

Where brittleness is unobjectionable, we use a collodion consisting of nitrocellulose dissolved in ether and alcohol; but where flexibility is desired, we use a collodion containing also nitroglycerin, in the proportion, preferably, of about two parts of nitroglycerin to one part of nitrocellulose, and dissolve them in ether and alcohol to which has been added a small proportion of acetone. Communication trains molded from

material made with the nitroglycerin-nitrocellulose collodion are less brittle than those made with the nitrocellulose collodion.

Two illustrative compositions are herewith submitted:

|                | I.  | 60     |
|----------------|-----|--------|
| Black powder   | 750 | grams. |
| Nitrocellulose | 250 | grams. |
| Ether          | 500 | cc.    |
| Alcohol        | 250 | cc.    |

  

|                | II.               | 65     |
|----------------|-------------------|--------|
| Black powder   | 750               | grams. |
| Nitrocellulose | 88 $\frac{1}{2}$  | grams. |
| Nitroglycerin  | 166 $\frac{2}{3}$ | grams. |
| Ether          | 300               | cc.    |
| Alcohol        | 150               | cc.    |
| Acetone        | 16                | cc.    |

It will be understood that in the drying operation, the solvents almost entirely escape, and that any suitable known means 75 may be employed to recover the solvents for reuse.

Heretofore great difficulty has been experienced in the manufacture of black powder pellets, in getting them so hard that 80 they will resist the shock of acceleration when a shell is fired from a gun. This result heretofore has been sought by molding under exceedingly heavy pressure. By 85 modifying the black powder composition by the addition of collodion, not only is sufficient fluidity imparted to the composition to permit the manufacture of the pellets by the advantageous method described, but the resultant pellets have such physical qualities 90 that they may be depended upon to resist the shock of acceleration on firing.

In claiming black powder, we refer to the usual composition of niter, sulfur and charcoal, the proportions of which do not 95 vary much from 75, 10 and 15 per cent. respectively.

While we believe that cementing black powder dust into masses by means of a collodion to be new, our invention also involves 100 the discovery that the manufacture of perforated pellets, for use in powder communication trains, of the specified composition is a non-obvious use of the composition that produces certain beneficial results and 105 peculiar advantages that would not charac-

terize the use of the composition in the manufacture of any other kind of explosive product.

It will be understood that in claiming 5 "pellets" we do not mean to exclude a mass long enough to form a complete powder train.

While the pellets must be dried, a special 10 drying operation is not indispensable, inasmuch as drying will be incidental to ordinary exposure to the atmosphere.

Having now fully described our invention, what we claim and desire to protect by Letters Patent is:

15. 1. As a new explosive product for use in powder communication trains, a perforated pellet comprising a mixture of black powder and a collodion.
20. 2. As a new explosive product for use in powder communication trains, a perforated pellet comprising a mixture of black powder and a collodion, the percentage of black powder exceeding that of the collodion.
25. 3. As a new explosive product for use in powder communication trains, a perforated pellet comprising a mixture of black powder, nitrocellulose and nitroglycerin.
30. 4. As a new explosive product for use in powder communication trains, a perforated pellet comprising a mixture of black powder and a collodion in the proportion of approximately three parts of black powder and one part of the collodion.
35. 5. As a new explosive product for use in powder communication trains, a perforated pellet comprising a mixture of black powder and a collodion in the proportion of approximately three parts of black powder and one part of the collodion, the collodion containing nitrocellulose and nitroglycerin.
40. 6. As a new explosive product for use in powder communication trains, a perforated pellet comprising a mixture of black powder and a collodion, the collodion containing nitroglycerin and nitrocellulose, the percentage of nitroglycerin exceeding that of the nitrocellulose and the percentage of black powder exceeding that of the ingredients of the collodion combined.
45. 7. As a new explosive product for use in powder communication trains, a perforated pellet comprising a mixture of about nine parts of black powder, about two parts of nitroglycerin and about one part of nitrocellulose.
50. 8. As a new explosive product, black powder dust cemented together into masses by means of a collodion.
55. 9. As a new explosive product, black powder dust cemented together into masses by means of a collodion containing nitrocellulose and nitroglycerin.
60. 10. A mixture of black powder and col-

lodion perforated and shaped to form a pellet adapted for use in communication 6 trains, the same having the physical qualities required to enable it to resist the shock of acceleration on firing.

11. As a new explosive product, black powder dust in a predominating proportion 70 cemented together into masses by means of a substantially smaller proportion of a collodion.

12. The process of making an explosive product which comprises mixing a preponderating proportion of black powder dust with a relative small proportion of a collodion dissolved in a suitable solvent, and cementing the ingredients while plastic into its final shape.

13. The process of making perforated pellets of explosive powder for use in communication trains, which comprises mixing black powder with nitrocellulose dissolved in a volatile solvent, pressing the mixture 85 into tubular form, cutting the tubes to length, and drying.

14. The process of making perforated pellets of explosive powder for use in communication trains, which comprises mixing black powder with nitrocellulose and nitroglycerin dissolved in ether, alcohol and acetone, pressing the mixture into tubular form, cutting the tubes to length, and drying.

15. The process of making perforated pellets of explosive powder for use in communication trains of sufficient hardness to resist the shock of acceleration on firing, which comprises imparting temporary fluidity to the black powder by mixing it with nitrocellulose dissolved in a volatile solvent, exuding the same under suitable pressure to form an elongated mass, and cutting the same to the desired length.

16. The process of making perforated pellets of explosive powder for use in communication trains, which comprises mixing black powder with nitrocellulose dissolved in ether and alcohol in suitable proportion 110 to form a plastic mass and pressing the powder into an elongated perforated form.

17. The process of making perforated pellets of explosive powder for use in communication trains, which comprises mixing black powder with nitrocellulose and nitroglycerin dissolved in ether, alcohol and acetone in suitable proportion to form a plastic mass and pressing the powder into an elongated perforated form.

In testimony of which invention, we have hereunto set our hands, at Wilmington, Delaware, on this 7th day of June, 1918.

FRANCIS I. DU PONT.  
ERNEST DU PONT.